

# UNITED STATES PATENT OFFICE.

CUNO WERNER, OF PHILADELPHIA, PENNSYLVANIA.

## IMPROVEMENT IN COMPOSITIONS FOR DRESSING LEATHER.

Specification forming part of Letters Patent No. 12,171, dated January 2, 1855.

*To all whom it may concern:*

Be it known that I, CUNO WERNER, of the city and county of Philadelphia, in the State of Pennsylvania, have invented a new and useful Combination of Matter to be used in Dressing Leather; and I do hereby declare that the following is a full, clear, and exact description thereof.

The nature of my invention consists in the employment of a new compound to be applied to leather, after it is tanned and dried, in place of tanners' oil and tallow, which are generally used, for the purpose of rendering it more flexible and merchantable.

To enable others to make and use my invention, I give the following description of the compound I use:

I take sixty pounds of a saturated infusion of oak-bark, or other substances from which tannin is generally extracted. To this I add forty pounds of common train-oil and thoroughly incorporate the mixture by stirring and agitating it until it acquires the consistency of thick cream. I then add sixteen pounds of rosin, previously melted and incorporated with four pounds of hog's lard, and, finally, I mix with the above one ounce of creosote to preserve the compound from molding. The above proportions are those I find best in practice; but they may be slightly varied.

The invention is especially applicable to the dressing or dubbing of calf-skins for boots and

shoes, or what is generally called "upper-leather." To the composition of oil and tallow which is generally used my compound presents many advantages: first, on the ground of economy, as the comparative cheapness of the principal ingredients I use makes a saving of from thirty to fifty per cent., according to the market; secondly, by the use of the saturated infusion of bark combined with oil and rosin the composition strikes deeper and quicker into the leather than the usual dressing of oil and tallow. It dries quicker, softens the leather, and renders it more pliable. If the leather is to be colored black, it receives the coloring-matter more readily and with less labor. The lard is used to facilitate the melting of the rosin, and the creosote preserves it from mold.

Having thus fully described my invention, what I claim as new, and desire to secure by Letters Patent, is—

The use or employment of a compound for dressing leather, composed of a saturated infusion of oak-bark, (or other substances affording tannin,) train or fish oil, rosin, hog's lard, and creosote, compounded and combined as herein set forth, and for the purposes specified.

In testimony whereof I have hereunto signed my name this 9th day of November, 1854.

CUNO WERNER.

Witnesses:

CHAS. EVERETT,  
SAML. GRUBB.